

## UNITED STATES PATENT OFFICE

2,564,661

## STEEL PLATING METHOD

Arthur Arent, Fort Dodge, Iowa

No Drawing. Application January 10, 1946,  
Serial No. 640,388

4 Claims. (Cl. 117—130)

1

This invention relates to the art of bonding metallic surfaces or coatings to metal objects such as steel or iron, and more particularly relates to a cold-plating method of bonding metallic antimony on steel or iron.

In many instances, it is desirable to surface-coat steel and iron objects to render their exposed surfaces corrosion resistant. Antimony has been known to be highly satisfactory for this purpose, but in the past, the only satisfactory carriers for the antimony have been volatile, inflammable compositions, which present a fire and health hazard.

It is an object of the present invention to provide a simple, economical and efficient process for causing a deposition of metallic antimony in commingled union with exposed steel and iron surfaces.

Another object of this invention is to provide a cold-plating process for applying antimony plating to steel or iron, in which the plate forms an integral body with the steel and iron and contains few, if any, surface pinhole openings.

Still another object of this invention is to produce antimony-plated iron or steel having a high degree of corrosion resistance and which plating metal may be combined with a silicate composition to produce an integral coating having a glossy appearance.

Still another object of this invention is to provide an antimony-plating process by which a succession of integrally bonded plates can be formed in commingled union with the surface of steel or iron objects.

Other objects reside in the provision of novel steps and treatments, all of which will be fully explained in the course of the following description.

The present invention resides in the discovery that when an antimony-carrying brine is applied to clean iron or steel surfaces a reaction results which forms a commingled union of antimony with the iron or steel. The surface deposit, so formed, is a continuous layer or film, which is substantially, if not entirely, free from pinhole openings, and is formed integrally with the base metal. Likewise, if desired the clean metallic surface may be initially coated with water glass, after which the antimony-carrying solution is applied to the silicate surface and reacts with it and the underneath metal to form a glossy integral surface coating.

With this understanding of the general nature of the present invention, typical operations will be cited to provide a better understanding of

2

the practice of the invention. In the first of these a piece of steel was suitably cleaned as by sand blasting and the coating composition was applied to the cleaned surface by brushing.

5 This composition was formed by introducing one pound of common salt (NaCl) into one pint of rain water. This mixture was stirred to dissolve the salt and the excess salt was allowed to remain. One-half pound antimony trichloride (crystals) was added to the brine and stirred until the antimony was dissolved. This coating was allowed to dry thoroughly before rinsing with water.

It frequently is desirably to apply a plurality 15 of such coatings and this can be done in such a way that one coat or plate bonds with the next to form an integral structure of the type previously described. To this end, the second coating is applied over the first after it is dry, but before

10 it has been rinsed. The second coat is allowed to dry and if it is to be the final coat, is rinsed as aforesaid, or if it is to be an intermediate coat, the third coating also is applied before rinsing, and so on.

20 While I prefer to employ sodium chloride in preparing the brine of the treatment, it is possible to obtain satisfactory results by using other chlorides, such as potassium chloride or calcium chloride, in forming the brine.

25 In another test operation a piece of clean steel was initially coated with a solution of commercial water glass (sodium silicate). If desired, the sodium silicate solution may be thinned with distilled or rain water before coating the metal as aforesaid. After drying this base coating, the antimony-carrying brine is applied thereto as by brushing, or immersion, and when this second coating has dried, it is rinsed to complete the treatment.

30 As in the previous example, a plurality of coatings may be applied to the base coating by omitting the rinsing step until the final coating has been applied. The coating is relatively thick and there is no apparent division between the

35 antimony layer and the base metal, although intermediate these there is a layer which apparently is a mixture of both metals. The glass-like deposit which is intermingled with the metallic antimony is substantially or entirely free from pinhole openings and is water insoluble, and hence makes an excellent preservative for the base metal surface which otherwise would be exposed.

40 In the formation of all the aforesaid coatings, a film or residue, which apparently is oxide, in

that it has all the appearance and characteristics of oxide, forms at the surface when the coating is dry and has adhesive properties which are particularly suited for the reception of other coatings or finishes, such as paints or lacquers when such finishes are desired.

Consequently, in industrial application, railway car bodies, automobile bodies, fuel storage tanks and many similar objects may be treated to render the metal resistant to the deteriorating effects of salt or other corrosive atmospheres and then painted or lacquered to produce the desired ornamental effects.

In the foregoing description, I have referred to the use of rain water or distilled water as best results will be obtained when the aqueous medium is free from salts, such as those carried in many domestic water systems. However, it should be understood that any brine, when its salt content is at or near the saturation point, will be satisfactory for most purposes. Likewise, I prefer to use anhydrous antimony trichloride in preparing the treatment solution, but antimony chloride or, in fact, metallic antimony obtained from any source and dissolved in the brine solution will give workable results. Best results are obtained when the anhydrous antimony trichloride is introduced in the amount of four pounds per gallon of brine used, but workable results can be obtained by using lesser amounts.

While I have used the term "cold-plating process" in the specification to indicate the absence of heat or electric current in the treatment, as normal room temperatures are satisfactory, I do not intend such definition to exclude the use of hot solutions when they are needed for any other reason. In the various drying steps aforementioned, natural drying may be used, but if it is desired to accelerate the action, heating or other types of artificial drying may be used.

If the plating operation utilizes an immersion treatment, best results will be obtained if the material under treatment is submerged for an interval of at least three minutes. If a brushing action is used, every part of the surface

should be wet brushed several times before permitting it to dry.

What is claimed is:

1. The process for treating ferrous metal surfaces which comprises applying water glass to the surface to be coated, wetting the water glass surface after drying with a strong chloride solution carrying antimony dissolved therein for an interval sufficient to induce a surface reaction between antimony, the ferrous metal and water glass constituents, and drying the surface so reacted after metallic antimony has deposited on said surfaces.

2. The process for treating ferrous metal surfaces which comprises applying an alkali metal silicate solution to the surface to be coated, wetting the coated surface after drying with a strong solution having antimony ions and an excess of chloride ions therein for an interval sufficient to induce a surface reaction between antimony, the base metal and water glass constituents, and drying the surface so reacted after metallic antimony has deposited on said surfaces.

3. A process as defined in claim 2, in which the alkali metal silicate solution is formed by introducing sodium silicate in rain water.

4. A process as defined in claim 2, in which the alkali metal silicate solution is formed by introducing sodium silicate in distilled water.

ARTHUR ARENT.

30

#### REFERENCES CITED

The following references are of record in the file of this patent:

35

#### UNITED STATES PATENTS

| Number    | Name    | Date          |
|-----------|---------|---------------|
| 1,186,217 | Mark    | June 6, 1916  |
| 1,207,218 | Roux    | Dec. 5, 1916  |
| 1,436,729 | Scanlon | Nov. 28, 1922 |
| 1,770,828 | Arent   | July 15, 1930 |
| 2,271,706 | Morris  | Feb. 3, 1942  |
| 2,485,182 | Arent   | Oct. 18, 1949 |

40

#### OTHER REFERENCES

45 Mellor: Comprehensive Treatise on Inorganic and Theoretical Chemistry, 1929, vol. 9, page 474.